

June 21, 1938.

A. VOM BRAUCKE  
PROCESS FOR THE MANUFACTURE OF SHEETS, BANDS, TUBES,  
RODS, AND THE LIKE, AND IN PARTICULAR WIRE  
Filed Sept. 6, 1935

2,121,415



INVENTOR  
ADOLF VOM BRAUCKE,  
By Carl A. Hellmann,  
ATTORNEY.

## UNITED STATES PATENT OFFICE

2,121,415

PROCESS FOR THE MANUFACTURE OF  
SHEETS, BANDS, TUBES, RODS, AND THE  
LIKE, AND IN PARTICULAR WIRE

Adolf vom Braucke, Berge, Germany

Application September 6, 1935, Serial No. 39,496  
In Germany September 7, 1934

3 Claims. (Cl. 148—12)

In the manufacture of steel wire the process starts as a rule from wire made by rolling which is then drawn in one or more steps to the desired diameter. As, in the drawing, the danger of an excessive increase in hardness due to cold working and of resultant breaking of the wire may arise, the piece to be drawn is sometimes heat treated before the drawing and also between the various drawing stages. As regards this heat treatment, the so-called "patenting" of the wire is generally effected, that is to say, the wire is heated to somewhat above the  $Ac_3$  point which, according to the carbon content, lies at temperatures between  $900^{\circ}$  C. and about  $700^{\circ}$  C., and is finally quenched in a lead bath to temperatures of about  $500^{\circ}$  C. This heat treatment gives it a sorbitic structure with a fine grain. Owing to the fact that the heating is carried out for only a short time at or above the  $Ac_3$  point, the so-called normalizing range is arrived at in which the material assumes a fine grained structure.

Extensive research has now shown that the fine initial structure of wire which is to be drawn or rolled to a smaller cross-section has an unfavorable effect on the drawing process and the properties of the material, because the various grains can only be stretched to a well defined limit of length before they will break.

It has been found by my experiments that the long fibred wire has the best properties. Such a long fibred final structure can however be obtained only when starting from large grains. The coarse grained starting material is capable of the greatest decrease in cross-sectional area, that is to say, extensive cold working and thus, in addition to other advantages, makes a considerable economy in operation possible.

The invention relates to a process of heat treatment which will give the coarsest readily attainable grain formation in the material.

In the iron-carbon diagram illustrated in the drawing, the temperature ranges or zones characterizing the new process are designated I, II and III.

For obtaining as coarse a structure as possible, the wire, according to its carbon content and its cross-section is, in accordance with the invention, quickly brought to a temperature substantially above the  $Ac_3$  point ( $800^{\circ}$  C.— $1300^{\circ}$  C.). At this temperature, the whole carbon content is in solid solution and the material acquires a coarse structure. From the range I, the wire is then quenched to a temperature within the temperature range II which, according to the carbon content, is from  $720^{\circ}$  C.— $1050^{\circ}$  C. and finally is

quenched in a lead, air, salt, oil, blubber, petroleum, tallow, acid or alkaline bath to a temperature within the range III ( $0^{\circ}$  C.— $720^{\circ}$  C.) and, if desired, down to room temperature. The temperature to be reached in the range I of the iron-carbon diagram depends upon the quenching temperature in range II. The temperature is always determined so that a structure is obtained which is as coarse grained as possible.

It has also been found that it is advantageous to heat up to the high temperature as quickly as possible. This appears to be due to the fact that thereby complete solution of the carbide is obtained more quickly than would otherwise be the case. The new process has the advantage that no undissolved lamellae of cementite from a previous heat treatment are left in the material, so that during the quenching (range III of the iron-carbon diagram) no cementite can agglomerate with cementite lamellae remaining from a previous treatment. It has also been established that with a heat treatment in accordance with the invention, the distribution of any foreign substances along the grain boundaries is more favorable than with the previously usual treatment. By rapid heating to the high temperature, there is no time for this substance to separate out at the new grain boundaries but it separates out in a harmless intracrystalline fashion.

Summarizing, extraordinary advantages have been revealed in the practice of the new process. One of the most important is that wire can be cold drawn to a much greater extent with the same ultimate tensile strength and the number of heat treatments can be reduced to a minimum. The number of torsions, alternating torsions and bends under test increased by approximately 100% by the use of the process in accordance with the invention.

The new heat treatment process is not confined to the manufacture of wire. It is most useful wherever the material is to be cold worked as, for example, in the manufacture of sheet metal, tubes, bands, rods and the like.

Where, previously, cold worked articles were heat treated, the heating was, for instance, carried to a temperature below the  $Ac_1$  point or to a normalizing temperature for the purpose of avoiding any undue hardening before the next cold drawing operation. By means of the heating to below the  $Ac_1$  point or by means of the normalizing only a fine grained structure results. On the other hand, the structure of the objects treated as now proposed is coarse grained and,

as I have found that a material having a coarse structure can be drawn out to a much greater extent with the same ultimate tensile strength, it is clear that the use of the new process is extraordinarily advantageous in the treatment of all cold worked materials.

I have found in particular that when the hyper-eutectoid and alloyed types of iron are treated as described, the carbon or the whole of the constituents of the alloy become very uniformly distributed. The coarse carbide formation which in the heat treatments heretofore known led to some extent to making the material unfit for use is restrained by the new process. Also, a single heat treatment of hyper-eutectoid materials ensures a complete destruction of the cementite.

The heat treatment will take place before the cold working of the material and, when this is carried out in stages it can be repeated a number of times. The finished cold worked objects can, as in prior practice, be subjected to a temperature in the  $\alpha$  or  $\gamma$  ranges. In this way, where it is required for the use to which it is to be put, its structure can be made finer. If the objects are to be drawn or rolled to a special hardness, the drawing or rolling process can be interrupted at a correspondingly early stage according to the desired hardness, so that after the necessary consequent cold working to the final size, the desired hardening will also be attained simultaneously therewith.

The new process is suitable in particular for iron alloys but it can also be used for the manufacture of cold worked articles of other metals.

I claim:—

1. In the manufacture of sheets, bands, tubes, rods, wire and the like by cold working of iron or steel alloys, the step of treating the material preparatory to its cold working, for the purpose

of providing it with a coarse-grained structure, which step comprises rapidly heating the material to a temperature depending upon its carbon content and lying within zone I (800° to 1300° C.), quenching the material to a temperature within zone II (720° to 1050° C.), holding the material at said latter temperature for such time as is required to attain a temperature within zone II, and quenching said cooled material to a temperature within zone III (0° to 720° C.).

2. A process for manufacturing sheets, bands, tubes, rods, wire and the like, which comprises subjecting the material to cold working in a number of stages and heat-treating said material both before and after at least one of said stages, said heat treatment comprising rapidly heating the material to a temperature depending upon its carbon content and lying within zone I (800° to 1300° C.), quenching the material to a temperature within zone II (720° to 1050° C.), holding the material at said latter temperature for such time as is required to attain a temperature within zone II, and quenching said cooled material to a temperature within zone III (0° to 720° C.).

3. A process for manufacturing sheets, bands, tubes, rods, wire and the like, which comprises rapidly heating the material to a temperature depending upon its carbon content and lying within zone I (800° to 1300° C.), quenching the material to a temperature within zone II (720° to 1050° C.), holding the material at said latter temperature for such time as is required to attain a temperature within zone II, and quenching said cooled material to a temperature within zone III (0° to 720° C.), cold working said heat treated material, heating said cold worked material to a temperature below the  $Ac_1$  point and cooling said material in air.

ADOLF vom BRAUCKE. 40